

May 26, 1931.

H. F. TIELKE

1,807,453

ROLLING MILL PIERCING POINT, PLUG, AND GUIDE, AND METHOD OF MAKING SAME

Filed Aug. 23, 1929



*Fig. 1*



*Fig. 2*

Inventor

HOMER F. TIELKE

*Rickey & Watts*  
By

Attorneys

## UNITED STATES PATENT OFFICE

HOMER F. TIELKE, OF CLEVELAND, OHIO

ROLLING MILL PIERCING POINT, PLUG AND GUIDE, AND METHOD OF MAKING SAME

Application filed August 23, 1929. Serial No. 387,910.

This invention relates to steel alloys and to methods of heat treating the same. It also relates to articles for use in rolling mills such as piercing points, plugs and guides and other parts which are subjected to high compressive and frictional loads.

Heretofore such enumerated articles have usually been made of steel alloys containing chromium, and nickel but have not been satisfactory for the severe uses and service conditions to which they are subjected, this being particularly true in piercing points. Such material has been characterized by brittleness which often resulted in breakage of the articles before they had been worn out, and instances are known where such articles broke after but very little use. Moreover, the prior art articles have exhibited a tendency to wear out quickly.

By the present invention these previous disadvantages have been overcome and articles such as rolling mill piercing points, plugs, guides and other parts subjected to similar service conditions have been made which are not so subject to failure due to brittleness as the prior art articles, and which can be used repeatedly and for many times the amount of service given by the prior art articles.

According to the present invention a high carbon steel alloy is employed containing between about .75% and about 1.5% of carbon, between about 16% and about 19% of chromium and between about 2% and about 4% of cobalt. Nickel may also be present in the alloy in amounts of between about .4% and about 2% if desired. Tungsten may be present in the alloy in amounts up to about 2% if desired but satisfactory results have been obtained without the presence of tungsten. A preferred composition is a steel alloy containing about .80% of carbon, about 17% of chromium, about 35% of cobalt and about .60% of nickel.

In adapting alloys of this invention to use in such articles as piercing points, plugs, guides and the like, the alloy is preferably cast in a sand mold as nearly to size as possible and the casting is then ground to remove roughness and to bring the casting to size when necessary. Then the casting is heat

treated to bring about micro-structure which is characterized by consisting of homogeneous dendritic material of substantially uniform hardness. This may be accomplished by heat treating the casting as follows:

The casting is heated up to about 2250° F. for a period of time sufficient to insure that the interior of the casting has been brought to substantially such temperature. With piercing points a period of about five minutes at a temperature of 2250° F. is sufficient for this purpose but it will be understood that this length of time will depend somewhat on the size of the article being heated and the number of articles being heated at the same time. After the casting is thoroughly heated to about 2250° F. it is allowed to cool in air to room temperature, after which it is re-heated to between about 1400° F. and about 1800° F. and then quenched in oil at room temperature. The quenched article is then heated at a soaking temperature at about 1200° F. for a considerable period of time, about six hours having been found to be satisfactory for piercing points, rolling mill plugs and the like.

Articles composed of the foregoing alloys when treated according to the foregoing methods possess a micro-structure which is characteristically dendritic and martensitic, resembles tool steel as to grain size, and is homogeneous and of substantially uniform hardness throughout. It is characterized also by the absence of grains surrounded by grain boundary material of a markedly different hardness which is characteristic of the material in the as-cast condition.

I believe that when alloys of the foregoing composition are cast the higher melting point constituents are surrounded by grain boundary material of a different hardness and that the step of heating to about 2250° F. or well above the upper critical range of the alloy results in bringing about a dissolving action which removes much of, if not all, the grain boundary material. The cooling in air is at such a rate that the latter material does not precipitate out of the solid solution and the re-heating step which is carried out above the upper critical range of the alloy results,

in part at least, in a refining of the structure of the casting which structure is retained and prevented from grain growth by the oil quenching step. The final heating is carried out at such a temperature that the previously refined grains are prevented from material growth and any casting strains which may remain in the casting are removed and the structure is made more nearly uniform in 10 hardness and homogeneous in nature.

Articles made of the foregoing composition and by the foregoing heat treatment are also characterized by a high hardness coupled with a uniformity of hardness throughout, 15 that is, by the absence of parts which are much softer than other parts.

In the drawings accompanying and forming a part of this application,

Figure 1 shows the metalographic structure at about 800 magnification of an unheat-treated casting having the above mentioned preferred composition;

Figure 2 is a view of the same material at the same magnification but taken after the 25 material of Figure 1 had been heat treated according to the foregoing method.

Having thus described my invention so that those skilled in the art may be enabled to practice the same what I desire to secure 30 by Letters Patent is defined in what is claimed, it being understood that variations and changes in the composition of the alloy or in the steps of the method may be made without departing from the scope of my invention as claimed.

What is claimed is:

1. A steel alloy containing between about 17% and about 18% of chromium, about 3% of cobalt and between about .4% and 1.5% 40 of nickel, and having a structure characteristic of such an alloy which has been heated in cast form to about 2250° F. for about five minutes, cooled slowly, reheated to between about 1400° F. and about 1800° F., quenched and reheated at about 1200° F. for several hours.

2. A heat treated steel alloy article having a microstructure characteristic of high carbon steel containing between about 16% 50 and about 19% of chromium and about 2% and about 4% of cobalt, which has been heated to about 2250° F. for about five minutes, cooled slowly, reheated to between about 1400° F. and about 1800° F. and quenched and then reheated to about 1200° F. for about six hours.

3. A heat treated steel alloy article having a microstructure characteristic of high 60 carbon steel containing between about .75% and about 1.5% of carbon, between about 16% and about 19% chromium and between about 2% and about 4% of cobalt, which has been heated to about 2250° F. for about five 65 minutes, cooled in air, reheated to about 1800

degrees F. and quenched and then reheated to about 1200° F. for about six hours.

4. A heat treated steel alloy article having a microstructure characteristic of high carbon steel containing between about .75% 70 and about 1.5% of carbon, between about 16% and about 19% of chromium and between about 2% and about 4% of cobalt, and between about .4% and about 2% of nickel, which has been heated to about 2250° F. 75 for about five minutes, cooled in air, reheated to about 1800° F. and quenched and then reheated to about 1200° F. for about six hours.

5. The method of heat treating a steel alloy casting containing between about .75% and about 1.5% of carbon, between about 16% and about 18% of chromium and between about 2% and about 4% of cobalt, which comprises heating the casting to about 2250° F. until heated throughout, cooling the casting slowly, reheating to about 1800° F. and quenching, and heating at about 1200° F. for several hours.

6. The method of heat treating a steel alloy casting containing from about .75% to about 1.5% of carbon, from about 16% to about 18% of chromium and from about 2% to about 4% of cobalt which comprises heating the casting at such a temperature above its upper critical range and for a sufficient length of time to bring into solid solution a major part of the grain boundary material, cooling the casting in a manner to retain such dissolved grain boundary material in solid solution, reheating the casting to a temperature above the upper critical range sufficiently long to bring about a refining of the grain structure, quenching the refined structure, and then heating the casting at such a temperature and for a sufficiently prolonged time to produce a dendritic homogeneous structure of substantially uniform hardness throughout.

7. A heat treated rolling mill piercing point, plug or guide composed of a steel alloy containing between about .75% and about 1.5% of carbon, between about 16% and about 18% of chromium and between about 2% and about 4% of cobalt and having a microstructure characterized by being dendritic, homogeneous and of substantially uniform hardness throughout, and having a microstructure characteristic of a steel of the said composition which has been heated to about 2250° F. for about five minutes, cooled in air, reheated between about 1400° F. and about 1800° F., quenched and reheated at about 1200° F. for several hours.

In testimony whereof I hereunto affix my signature this 20th day of August, 1929.

HOMER F. TIELKE.